

# UNITED STATES PATENT OFFICE

2,138,023

## METHOD OF TREATING ANODIC COATINGS ON MAGNESIUM AND ITS ALLOYS

Robert W. Buzzard, Kensington, Md., and James  
H. Wilson, Washington, D. C.

No Drawing. Application November 14, 1935,  
Serial No. 49,758

3 Claims. (Cl. 148—6)

(Granted under the act of March 3, 1883, as  
amended April 30, 1928; 370 O. G. 757)

This invention relates to the heat treatment of  
anodically formed coatings on magnesium and its  
alloys and has among its objects to increase the  
durability and the protective characteristics of  
the film.

The article to be treated according to our in-  
vention is first coated in a suitable anodizing bath,  
washed free of solution, and allowed to dry.

The coated article may then be subjected to  
one of the various contemplated modes of carrying  
out the present invention. It may, for example,  
be heated in an oven or furnace at some tempera-  
ture above 100° C., the upper limit of temperature  
being safely below the fusion point of the metal  
and the duration of the heating dependent upon  
the temperature used. In general, the lower the  
temperature the longer should be the period of  
heating.

Another way of realizing the benefits of our in-  
vention is to dip the anodically coated article in  
melted paraffin or in some other combustible  
organic substance that will adhere to the article  
and then heating as above described, or the or-  
ganic substance may be ignited and allowed to  
burn off. Still another method is to heat the  
coated article in an open flame or in the presence  
of a gaseous hydrocarbon.

All of these methods produce similar results.  
The treatment makes the film less soluble and  
usually lightens the color thereof, the greater  
color changes being effected when heat is applied  
in the presence of a hydrocarbon.

This invention may be manufactured or used  
by or for the Government of the United States of  
America for governmental purposes without the  
payment of any royalty thereon or therefor.

### We claim:

1. A method of treating an anodically formed  
film on magnesium and its alloys, which comprises  
heating the coated metal at a temperature above  
100° C. and lower than the fusion point of the  
metal in a hydrocarbon.
2. A process of treating an anodically formed  
film of magnesium and its alloys, which comprises  
applying paraffin to said film and removing a  
substantial portion of the paraffin by heating the  
coated metal to a temperature above 100° C. and  
lower than the fusion temperature of the metal.
3. A method of treating an anodically formed  
film on magnesium and its alloys, which comprises  
applying a combustible hydrocarbon to the film  
on said metal and igniting the hydrocarbon.

ROBERT W. BUZZARD.  
JAMES H. WILSON.